

# UNITED STATES PATENT OFFICE.

JOSEPH W. TAYLOR, OF NEW WATERFORD, OHIO.

## HOT-WORK ARTICLE.

1,282,981.

Specification of Letters Patent. Patented Oct. 29, 1918.

No Drawing.

Application filed March 9, 1917. Serial No. 153,652.

*To all whom it may concern:*

Be it known that I, JOSEPH W. TAYLOR, residing at New Waterford, in the county of Columbiana and State of Ohio, a citizen 5 of the United States, have invented or discovered certain new and useful Improvements in Hot-Work Articles, of which improvement the following is a specification.

My invention relates to new and useful 10 improvements in hot-work tools, implements or other articles of manufacture made of steel, and which, in practice, are subjected to frequent wide variations in temperature. Tools of this sort include dies, punches, or 15 other shaping or cutting implements used to operate upon hot metal, glass, etc., while puppet valves for internal combustion engines are examples of engine elements which are subjected to such temperature conditions, 20 and which, to withstand the wear to which they are subjected, should be hard and tough.

The object of my invention is to provide 25 steel hot-work articles, of the character just explained which will be hard and tough and which will resist fire cracking to an extent not heretofore realized.

My invention results from my discovery 30 that the addition of certain percentages of carbon and chromium to steel will produce an alloy which will accomplish the above stated object of my invention, and that the further addition to such steel of certain percentages of an anti-fatiguing element will 35 produce an alloy which is still better for the stated purpose. By anti-fatiguing is meant an element, which, when added to an alloy, will increase its capability of resisting high strains, particularly repeated strains, 40 whether applied mechanically or resulting from a physical phenomenon such as changes in temperature.

The alloy which I provide and which I have found to be hard and tough and to resist fire cracking to a far greater extent than any alloy heretofore produced for hot-work articles is essentially a high carbon chromium steel, the carbon content being from about 1.50% to 3.00% and the chromium 50 3.00% to 7.00%. While, good results may be obtained by hot-work articles made of such an alloy uncombined with additional ingredients other than the usual impurities found in steel, I find that still better results 55 may be had by using such alloy further combined with not less than about .50% of an

anti-fatiguing element such as nickel or vanadium. The best results, however, are obtained by a steel alloy having percentages of carbon and chromium falling within the above stated limits and also containing both nickel and vanadium, the nickel content ranging from about .50% to 3.50% and the vanadium content from about .50% to 2.00%. 60

The chemical analysis of a specific example of the hot-work steel alloy which I provide shows the following elements present in the percentages stated: carbon 2.25%, chromium 4.66%, nickel .61%, vanadium .97% and manganese .41%. The Brinell hardness of this steel as cast was 418, and it was sufficiently tough to enable it to be forged satisfactorily. Several forging dies were constructed of this steel alloy, and, 70 after having been kept in continuous service for a period of more than three months, showed no signs of fire cracking.

The hot-work steel alloy which I provide may be manufactured by the usual well known process for making similar steel alloys. 75

When the alloy is hardened from a temperature of from about 750° to 1000° C. it exists in a very hard condition tending to 80 toward brittleness, that is to say in a martensitic condition containing excess carbids. When hardened from a temperature above 1025° C., more particularly from 1100° C., it exists in a file-hard but dynamically soft 85 or austenitic condition having a Brinell hardness of from about 286 to 302. This condition is unchanged upon reheating until a temperature of about 550° C. is reached, at which point there is a marked increase in 90 hardness—a conversion into a martensitic condition plus an immediate partial sorbitic change. Such change gives a much desired 95 combination of hardness and toughness which cannot be obtained in desired proportions by simply hardening from about 850° C. and drawing. 100

This phenomenon of the increase in hardness on drawing appears to be a delayed critical range which is liberated on drawing, as shown by the fact that on heating to the increase hardness range an exothermic reaction takes place, that is to say the specimen "glows" in a manner commonly observed on passing ordinary steel through 105 the recalescence or cooling range. This re-glowing or heating is a phenomenon which. 110

to the best of my knowledge, is not characteristic of other steels or steel alloys.

From the foregoing explanations of the physical changes which characterize my alloy when subjected to various heat treatment, it will be observed that the alloy possesses physical properties different from those of any other steel alloy.

I claim as my invention:

- 10 1. A hot-work article formed of a steel alloy containing from about 1.50% to 3.00% carbon, and from about 3.00% to 7.00% chromium.
- 15 2. A hot-work article formed of a steel alloy containing from about 1.50% to 3.00% carbon, from about 3.00% to 7.00% chromium, and not less than about .50% of an anti-fatiguing element.
3. A hot-work article formed of a steel

alloy containing from about 1.50% to 3.00% 20 carbon, from about 3.00% to 7.00% chromium and not less than about .50% each of nickel and vanadium.

4. A hot-work article formed of a steel alloy containing from about 1.50% to 3.00% 25 carbon, 3.00% to 7.00% chromium, .50% to 3.50% nickel, and .50% to 2.00% vanadium.

5. A hot-work forging die formed of a steel alloy containing from about 1.50% to 3.00% carbon, and from about 3.00% to 7.00% chromium.

In testimony whereof I have hereunto set my hand.

JOSEPH W. TAYLOR.

Witnesses:

JOS. W. WEITZENKORN,  
PAUL N. CRITCHLOW.

Copies of this patent may be obtained for five cents each, by addressing the "Commissioner of Patents, Washington, D. C."